

April 15, 1930.

L. KIRSCHBRAUN

1,754,771

PROCESS OF MAKING CURVED ROOFING ELEMENTS AND PRODUCT THEREOF

Original Filed Oct. 1, 1923

Fig. 1.



Fig. 2.



Fig. 3.



Fig. 4.



Fig. 5.



Witness:

Stephen & Roberta

by

Inventor:  
Lester Kirschbraun  
Frank L. Belknap  
G. G.

## UNITED STATES PATENT OFFICE

LESTER KIRSCHBAUM, OF CHICAGO, ILLINOIS, ASSIGNOR TO THE PATENT AND LICENSING CORPORATION, OF BOSTON, MASSACHUSETTS, A CORPORATION OF MASSACHUSETTS

## PROCESS OF MAKING CURVED ROOFING ELEMENTS AND PRODUCT THEREOF

Application filed October 1, 1928, Serial No. 665,805. Renewed December 24, 1927.

This invention relates to improvements in a process of making curved roofing elements and the product produced thereby and refers more particularly to the production of a roofing element or structure comprising convex and concave cylindrical segments which may be laid in a manner overlapping so as to simulate the well known Spanish tile or other tile-like ornamental roof structures. Some 10 of the subject matter of this application is also disclosed generically in Patent No. 1,612,776, granted to me December 28, 1926. Such subject matter which is generic to both the said patent and this application is dis- 15 claimed in this application.

Heretofore roofing elements have been made of paper or rag felt saturated with asphalt, coated and carrying an ornamental grit surfacing. These elements have taken 20 the form of shingles or similar flat structures and present, when placed on the roof, a flat monotonous, and to some, an inartistic, appearance.

Among the objects of the present invention 25 are to produce a roofing element devoid of this flat appearance, and having broken contours such as may be obtained from curved structures and curved surfaces, both of convex and concave form overlapping to produce a covering, among others, similar to that 30 which results in placing clay tile and having the shadow lines in relief caused by structures having raised contours; to produce a roofing element which, when laid, gives the 35 roof the effect pointed out yet possesses properties of lightness which does not require the heavy supporting structure which 40 is necessary for the placement of a clay tile roof; to produce a structure which, while 45 having the shape and other characteristics of clay tile, possesses toughness and flexibility so that breakage in transportation and handling is small; to provide a tile-like roofing element which is more or less flexible so 50 that it may accommodate itself to expansion and contraction and the effect of the elements; to provide a roofing element of fiber stock in which the curvature is inherent in the formation of the stock; to produce a 55 curved roofing element in contradistinction

to a flat one in which there will be no tendency for such element to flatten out due to internal fiber stress; and to produce a roofing element which is waterproof, weather- 60 proof and of substantial thickness and strength.

In the drawings:

Fig. 1 is a perspective view of my improved roofing element.

Fig. 2 is a perspective view of the cylindrical fibrous member from which the roofing element shown in Fig. 1 is cut. 65

Fig. 3 is a cross sectional view taken on the lines 3—3 of Fig. 1.

Fig. 4 is a perspective view of the assembled elements placed on a roof in overlapping relation. 70

Fig. 5 is a cross section of the roof as laid, taken on the lines 5—5 of Fig. 4.

Referring to the manner of making my improved product—I may first make an aqueous emulsion of asphalt with colloidal clay and water, or with similar colloidal agent, capable of producing a nonadhesive emulsion. The method of producing this emulsion is set 75 forth in issued United States Letters Patent No. 1,302,810, dated May 6, 1919, in patent issued to me. The emulsion may be made in batch or may be made by a continuous process. The asphalt or bituminous material 80 used in the emulsion should preferably be of relatively high melting point so that it may possess a maximum stability under the heat of the summer sun. I have found oxidized asphalts to be very satisfactory for this 85 purpose.

The paper stock which comprises the fibrous constituent of my roofing element, may be mixed papers, news, rags, kraft, in fact almost any paper is suitable for this purpose except that when it is desired to provide maximum strength and stiffness it is well to incorporate with such cheaper fibers as mixed papers, a substantial amount of kraft which is well hydrated so as to produce a slow stock 90 capable of imparting great stiffness and stability to the finished roofing element. After the fibrous stock has been prepared in the beaters in the usual way, there is added either to the beaters or the stuff chest, a pre- 95 100

determined quantity of the asphalt emulsion prepared as above stated. Sufficient emulsion is added so that the resulting stock when formed and dried is thoroughly impregnated with asphalt and is waterproof and weather resistant. Ordinarily 100 to 120 parts of asphalt, in emulsion form, to 100 parts of paper stock will be sufficient for this purpose. After the addition of the asphalt emulsion to the paper stock, a small amount of alum or other flocculating agent is added to the mixture in order to precipitate the dispersed particles of asphalt upon the fibrous stock.

The stock so prepared is fed to the well known wet machine, a brief description of which it is thought will suffice as it forms no part of the present invention. This wet machine is an ordinary wet machine which is used to make up heavy boards and differs only in being provided with a rotatable reel carrying a plurality of small make up cores or reels which may be successfully contacted with the wet sheet and upon which the web is picked up and formed into a cylindrical tube. When a tube of the desired thickness is formed, a reel is drawn or moved out of contact with the blanket, bringing the consecutive make up core into contact for the formation of the next fibrous tube. The make-up cores, with their fibrous tubes, are moved from the reel, inserted in the press to remove further quantities of water and then collapsed so that the fibrous tube with its contained asphalt may be removed therefrom.

It will be seen by this method of forming the fibrous tube from a wet web, that the fibers contained in the tube have thus accommodated themselves to a position of curvature, tending to retain the curved structure and presenting a maximum resistance to flattening out, thus distinguishing from laminated tubes or structures formed from flat sheets. In forming a tube by laminating previously prepared paper, the tendency is to elongate the fibers on the outer or convex surface while compressing the fibers on the inner or concave surface of the sheet, thus introducing stress which tends to relieve itself by resuming a flat position, in other words, flattening out. The method described of forming the tube from the wet web eliminates this tendency and eliminates the use of cementing mediums which are required in the laminating process just referred to.

The tubes thus formed are placed in a drying oven and subjected to a temperature of from 200 to 260 degs. F., the temperature being regulated so as to remove the water and cause the bitumen to coalesce and thoroughly impregnate the tube structure. This tube may be from 5" to 8" in diameter more or less; from  $\frac{1}{8}$  to  $\frac{1}{4}$ " thick; and of any convenient length.

After the tube is dried, it is then cut into longitudinal sectors representing say, one

half to one third of the periphery of the tube and it may be further cut transversely so as to produce a roofing element of any convenient length, say, from 12 to 18". In other words, I cut the tube into a plurality of cylindrical segments.

Referring now to the drawing, 1 represents a cylindrical segment cut in the manner just described from the cylindrical core or tube 2, this tube 2 having been previously formed in the manner above described. The cylindrical segments may now be placed upon a conveyor and passed through a bath of hot asphalt, the purpose of which is to coat both surfaces and all edges of the roofing element; preferably this asphalt will be oxidized petroleum residuum of approximately 200 to 240 degs. melting point and may be 25 penetration. As the roofing elements emerge from their bath of asphalt, there may be projected on the hot coating, grit particles of predetermined color. In some instances, these grit particles may be projected on the convex surface of the roofing element while in others the concave surface will receive the projected grit.

As will be seen in Fig. 3, the finished product will comprise a fibrous base 3 coated on either or both sides with the bituminous waterproof coating 4 and surfaced with the colored grit surfacing 5.

Instead of using oxidized asphalt as a coating, there may be employed colorable pitches such as stearine pitches and the like in which pigments are incorporated so as to impart a predetermined shade to the bituminous coating material. In such instances, it will be unnecessary to provide a grit surface as the ornamental effect will be included in the bituminous covering.

I claim as my invention:

1. A process of producing roofing elements having curved surfaces comprising sheeting a fibrous stock into a wet web, forming said sheeted fibrous stock into a tube from the wet web, drying the tube and slitting the same longitudinally and transversely into roofing elements of predetermined size and configuration.

2. A process of producing roofing elements having curved surfaces comprising sheeting a fibrous stock into a wet web, forming said sheeted fibrous stock into a cylindrical tube from the wet web, drying the tube and slitting same longitudinally and transversely into roofing elements of predetermined size and configuration.

3. A process of producing roofing elements having curved surfaces comprising sheeting a fibrous stock carrying a waterproofing medium into a wet web, forming said sheeted fibrous stock into a tube from the wet web, drying the tube, thereby causing the waterproofing medium to coalesce, and slitting same longitudinally and transversely into

70

75

80

85

90

95

100

105

110

115

120

125

130

- roofing elements of predetermined size and configuration.
4. A process of producing roofing elements having curved surfaces comprising sheeting a fibrous stock into a wet web, forming said sheeted fibrous stock into a tube from the wet web, drying and waterproofing the tube, and slitting same longitudinally and transversely into roofing elements. 70
5. A process of producing roofing elements having curved surfaces comprising sheeting a fibrous stock into a wet web, forming said sheeted fibrous stock into a tube from the wet web, drying the tube and slitting the same longitudinally and transversely into roofing elements, and coating said elements. 75
6. A process of producing roofing elements having curved surfaces comprising sheeting a fibrous stock into a wet web, forming said sheeted fibrous stock into a tube from the wet web, drying the tube and slitting the same longitudinally and transversely into roofing elements, coating said elements and imbedding therein a grit surfacing. 80
7. A process of producing roofing elements having curved surfaces comprising sheeting a fibrous stock into a wet web, forming said sheeted fibrous stock into a tube from the wet web, drying the tube and slitting the same longitudinally into roofing elements of predetermined size and configuration. 85
8. A process of producing roofing elements having curved surfaces comprising sheeting a fibrous stock into a wet web, forming said sheeted fibrous stock into a cylindrical tube from the wet web, drying the tube and slitting same longitudinally into roofing elements of predetermined size and configuration. 90
9. A process of producing roofing elements having curved surfaces comprising sheeting a fibrous stock carrying a waterproofing medium into a wet web, forming said sheeted fibrous stock into a tube from the wet web, drying the tube, thereby causing the waterproofing medium to coalesce, and slitting same longitudinally into roofing elements of predetermined size and configuration. 95
10. A process of producing roofing elements having curved surfaces comprising sheeting a fibrous stock into a wet web, forming said sheeted fibrous stock into a tube from the wet web, drying and waterproofing the tube, and slitting same longitudinally into roofing elements. 100
11. A process of producing roofing elements having curved surfaces comprising sheeting a fibrous stock into a wet web, forming said sheeted fibrous stock into a tube from the wet web, drying the tube and slitting the same longitudinally into roofing elements, and coating said elements. 110
12. A process of producing roofing elements having curved surfaces comprising sheeting a fibrous stock into a wet web, forming said sheeted fibrous stock into a tube from the wet web, drying the tube and slitting same into curved roofing elements devoid of internal fibrous strain and of grit surfacing. 115
13. Curved roofing elements cut on a longitudinal line of severance from a tube, comprising a fibrous base impregnated with waterproofing medium and devoid of internal fibrous stress. 70
14. A curved roofing element comprising a non-rigid fibrous base impregnated with a bituminous waterproofing medium, the fibres being disposed to eliminate internal strain, possessing the characteristics of having been formed in curved relation while wet. 75
15. Curved roofing elements produced by severing a tube longitudinally, comprising a fibrous base, the fibres being disposed to eliminate internal strain, and coated with a waterproof coating and an ornamental surfacing. 85
16. A process of producing roofing elements having curved surfaces comprising forming wet fibrous stock into a tube, drying, said tube and slitting same into roofing elements of predetermined size and configuration. 90
17. A process of producing roofing elements having curved surfaces comprising forming wet fibrous stock containing water repellent material, into a tube, drying said tube and slitting same into curved roofing elements devoid of internal fibrous strain and of pre-determined size and configuration. 95
18. A process of producing roofing elements having curved surfaces comprising forming wet fibrous stock into a tube, drying said tube and slitting same into roofing elements of predetermined size and configuration, and coating the surfaces and all edges of said roofing element with waterproof material. 105
19. A process of producing roofing elements having curved surfaces comprising forming wet fibrous stock containing water repellent material into a tube, drying said tube and slitting same into curved roofing elements devoid of internal fibrous strain and of pre-determined size and configuration, and coating surfaces and edges of said roofing element with waterproofing material. 110
20. A process of producing roofing elements having curved surfaces, comprising forming wet fibrous stock into a tube, drying said tube and slitting same into roofing elements of predetermined size and configuration, and coating the surfaces and all edges of said roofing element with waterproof material and imbedding in said waterproof material, particles of granular surfacing. 120
21. A process of producing roofing elements having curved surfaces, comprising forming wet fibrous stock containing water repellent material into a tube, drying said tube and slitting same into curved roofing elements devoid of internal fibrous strain and of grit surfacing. 125

pre-determined size and configuration, and coating surfaces and edges of said roofing element with water-proofing material, and imbedding in said waterproofing material, particles of granular surfacing.

22. A curved roofing element comprising a flexible fibrous base impregnated with a bituminous water-proofing material and devoid of internal fibrous stress.

10 23. A curved roofing element comprising a flexible fibrous base impregnated with a bituminous water-proofing material and devoid of internal fibrous stress, having a bituminous coating of water-proofing material covering said element.

15 24. The process of making roofing elements which comprises the steps of cutting the elements of suitable size and configuration from fibrous stock saturated with bituminous waterproofing material and in thereafter subjecting the saturated roofing elements to an application of bituminous coating material whereby to coat the exposed surface and seal the exposed edge of the saturated elements and in finally applying comminuted surfacing material to the thus coated elements.

LESTER KIRSCHBRAUN.